

Aug. 19, 1952

E. WEISS ET AL

2,607,655

STRIPED, CREPED CELLULOSE FABRICS WITHOUT MOIRE EFFECT

Filed July 29, 1949

EFFECT 1.



EFFECT 2.



INVENTORS.  
ERNST WEISS.  
KARL RISCH.  
BY  
*Ward Crosby Neal*  
Their ATTORNEYS.

## UNITED STATES PATENT OFFICE

2,607,655

STRIPED, CREPED CELLULOSE FABRICS  
WITHOUT MOIRÉ EFFECT

Ernst Weiss and Karl Risch, Wattwil, Switzerland, assignors to Heberlein Patent Corporation, New York, N. Y., a corporation of New York

Application July 29, 1949, Serial No. 107,426  
In Switzerland August 3, 1948

9 Claims. (Cl. 8—114.5)

1

This invention relates to a process for producing substantially parallel colored striped crepe-like effects on cellulose-containing fabrics and to products obtained therefrom.

It is known that shrunk effects on fabrics can be obtained by printing the fabric with a resist in the form of stripes and subsequently subjecting it to a caustic lye treatment whereby the areas to which the resist has not been applied shrink. It is also known that a similar result may be obtained by printing the lye on the fabric in the form of stripes. In both cases, an even crepe-like curling of the fabric surface is obtained. It has also been proposed to combine such shrinking effects with color printing. Printing of striped patterns with which the stripe-like shrunk areas are parallel, frequently produces undesirable effects, namely, moiré effects, giving rise to complaints in the trade.

The principal object of the present invention, accordingly, is to produce such substantially parallel colored stripe and crepe-like effects while avoiding the objectionable moiré effect.

The invention accordingly consists of the novel products as well as the novel processes and steps of processes according to which such products are manufactured, the specific embodiments of which are described hereinafter by way of example and in accordance with which we now prefer to practice the invention.

It has been discovered in accordance with our invention that the moiré effect can be eliminated by adjusting the width of the colored stripes, the distance therebetween, and the width of the shrunk and unshrunk areas.

We have found in accordance with our invention that the objectionable effects referred to may be overcome by printing a fabric with parallel spaced colored stripes, the fabric containing sufficient cellulose to produce a crepe effect when treated with a caustic shrinking agent capable of shrinking the cellulose and the fabric also having resistant stripes which are resistant to shrinkage as well as shrinkable stripes. The shrink-resistant stripes and shrinkable stripes are parallel to the colored stripes. The fabric is shrunk by applying caustic soda as a shrinking agent thereto. The shrinking agent is then removed from the fabric. The relation between the colored stripes, shrink-resistant stripes and the spaces between is in accordance with both of the following equations:

$$I \quad \frac{d}{c} \approx \frac{b}{a}$$

2

$$II \quad \frac{c+d}{a+b} \approx \frac{n}{2}$$

where  $a$  is the width of a colored stripe,  $b$  is the space between adjacent colored stripes,  $c$  is the width of a shrink-resistant stripe,  $d$  is the width of the space between adjacent shrink-resistant stripes, and  $n$  is an odd integer except 1.

Furthermore, in addition to the above mentioned relations, also no moiré effects will result when the width of the shrink-resistant stripes or the space between two such adjacent stripes is equal to the sum of the width of the colored stripe  $a$  and the space  $b$  between two such adjacent colored stripes or is an integral multiple of that sum, if the width of a shrink resistant stripe  $c$  is equal to the space  $d$  between adjacent shrink resistant stripes. This may be expressed by the following formulas

20 III

$$c=d$$

$$IV \quad \frac{c+d}{a+b} \approx 2k$$

where  $a$  is the width of a colored stripe,  $b$  is the space between adjacent colored stripes,  $c$  is the width of a non-shrinkable stripe,  $d$  is the space between adjacent non-shrinkable stripes, and  $k$  is any integer.

Upon shrinking such a fabric in the usual manner, a striped fabric is produced which does not exhibit the undesired moiré effect.

The accompanying drawings are intended to show the results of processes operating in accordance with the variant of the invention relating to the Equations I and II (Figure 1) and the results of processes not operating in accordance with this variant of the invention and which consequently produce the undesired moiré effects (Figure 2).

In these drawings,

Figure 1 represents a highly magnified fragment of a color stripe fabric printed with a resist running parallel to the parallel stripes of the fabric, the fabric having been prepared in accordance with the invention, and

Figure 2 shows a similar fabric with narrower colored stripes and with a resist printed in a manner so that the moiré effects appear.

Referring to Figure 1, it will be noted that the letter  $a$  is the width of a colored stripe,  $b$  is the spaced width between adjacent colored stripes,  $c$  is the width of a shrink resistant stripe,  $d$  is the width of the space between adjacent shrink resistant stripes.

55 In this figure it will be noted that the third

stripe from the left in the figure shows cross-hatching on either side thereof. This cross-hatching is intended to designate the area  $c$  referred to above and this area  $c$  extends all the way across the stripe mentioned. The same is true of all other stripes in both Figures 1 and 2, in which a portion of the cross-hatched area appears next to the colored stripe. In all such areas the resistant area  $c$  extends across the colored stripe. In this Figure 1 the fabric, unenlarged, has these dimensions:  $a=0.8$  mm.;  $b=1.6$  mm.;  $c=1.2$  mm., and  $d=2.4$  mm. Applying these dimensions to the Formulas I and II given above we have the following:

$$\frac{2.4}{1.2} \approx \frac{1.6}{0.8} \approx 2$$

and

$$\frac{1.2+2.4}{0.8+1.6} \approx \frac{1.5}{2} \approx \frac{n}{2}$$

Therefore,  $n=3$ . Where  $n$  equals 3, which is an odd integer other than 1, the resulting fabric does not show the moiré effect.

In Fig. 2,  $a=0.5$  mm.;  $b=1.2$  mm.;  $c=0.8$  mm., and  $d=1.0$  mm. Applying these figures to the above formulas we have:

$$\frac{1.0}{0.8} \neq \frac{1.2}{0.5}$$

and

$$\frac{0.8+1.0}{0.5+1.2} \approx \frac{1.06}{2} \approx \frac{n}{2}$$

Therefore,  $n$  equals 2.12 which is approximately 2, which is an even integer, and which will result in the moiré effect.

As Fig. 2 clearly shows, the shrink-resistant stripes in the zones marked A coincide at least approximately with the colored stripes, whereas in the region marked B they are in the intervals between every two colored stripes. After having been shrunk, a fabric made in accordance with Fig. 2 shows such regions A and B in respect of the shrunk and non-shrunk stripes and the colored stripes and the spaces therebetween. The alternating succession of such regions A and B is the cause of moiré effects.

In comparison to Fig. 2, no regions A and B are seen in Fig. 1 where there is a non-shrinkable stripe in between every two colored stripes and the one succeeding partly covers the colored stripe. In this case no, or only a slight moiré effect appears.

The following are examples of our process as we now prefer to practice it. In the first three of these examples the width of the stripes and spaces therebetween are in the relations of the equations

$$I \quad \frac{d}{c} \approx \frac{b}{a}$$

$$II \quad \frac{c+d}{a+b} \approx \frac{n}{2}$$

In the fourth, fifth and sixth examples the width of the stripes and spaces therebetween relate to the formulas

$$III \quad c \approx d$$

$$IV \quad \frac{c+d}{a+b} \approx 2k$$

It is to be understood that these examples are illustrative and that the invention is not to be restricted thereto except as indicated in the appended claims.

#### Example 1

A bleached and mercerized light weight fabric such as cotton muslin with 90 threads number 80 single per inch in the warp and 82 threads number 120 single per inch in the weft is printed in a stripe pattern with a vat dyestuff as for instance, Cibanon Black (Color Index 1172), the width of the stripe being 0.8 mm. and the inter-space between stripes being 1.6 mm. The fabric is then steamed, washed and dried under tension. Then a known water-soluble gum reserve, for instance, gum arabic, is printed on the fabric provided with the color print, in the form of stripes of 1.2 mm. in width, spaced at 2.4 mm. running parallel to the color stripes. Then the fabric is dried and subjected to the reaction of caustic soda of 38° Bé., whereby the areas not printed with the gum reserve shrink. Then the fabric is acidified with diluted sulfuric acid, washed until neutral, and dried. The relation of the width of a stripe to be shrunk to the space of two such stripes is equal to the relation of a color stripe space to the color stripe width. The mathematical relationship is expressed as follows in accordance with the Formulas I and II given above:

$$\frac{(d)}{2.4} \approx \frac{(b)}{1.2} \approx \frac{1.6}{0.8}$$

$$\frac{(c)}{0.8+1.6} \approx \frac{(d)}{2.4} \approx \frac{3.6}{2.4} \approx \frac{n}{2}; n \approx 3$$

This produces a fabric without moiré effects.

Coarser or finer striped patterns than those mentioned in Example 1 may be used; for instance, a very fine color stripe of 0.2 mm. width (a) and a space between adjacent color stripes of 1 mm. (b) may be used; the width of the shrink-resistant stripe is 0.5 mm. (c), and the space between adjacent shrink-resistant stripes, that is, the width of the stripes to be shrunk, is 2.5 mm. (d). Accordingly, in this case, substituting the figures in the Equations I and II given above

$$\frac{(d)}{2.5} \approx \frac{(b)}{1} \approx \frac{1}{0.2}$$

and

$$\frac{(c)}{0.2+1} \approx \frac{(c)}{0.5+2.5} \approx \frac{3}{2} \approx \frac{n}{2}; n \approx 5$$

Suitable effects may also be obtained with a stripe pattern with a color stripe width of about 1 mm. (a) and with a width between stripes of about 2 mm. (b); (c) in this case equals 1.5 mm. (a) equals 3 mm. Accordingly, substituting these figures in the above Formulas I and II

$$\frac{(d)}{3} \approx \frac{(b)}{1.5} \approx \frac{2}{1}$$

and

$$\frac{(c)+(d)}{2} \approx \frac{1.5+3}{1+2} \approx \frac{4.5}{3} \approx 1.5; n \approx 3$$

In the above and following examples, the resulting effects can be further modified by dyeing the fabric in the piece or by combining with any other desired printed pattern.

Instead of printing gum arabic on the face of the fabric as a gum resist in the above Example 1, a water-insoluble lacquer, for instance, a nitro-cellulose lacquer, can be printed on the reverse side of the fabric. In so doing, this nitro-cellulose lacquer is made up of the concentration of 240 gms. of nitro-cellulose to 748 cc. of a mixture of amylacetate, aethylacetate and ethyl-alcohol as a solvent and is applied in a well-known manner. The stripes of this lacquer on the back of the fabric occupy exactly the same position as the stripes of gum arabic occupy on the face of the fabric, but, of course, when such nitro-cellulose lacquer is applied, the gum arabic stripes are omitted. After washing the fabric, some of the lacquer remains on the fabric and gives a slightly stiffening effect to the printed areas. In addition, instead of applying the shrinking agent, namely, caustic soda, as indicated, such caustic may be printed onto the fabric in the form of stripes instead of by the resist printing above indicated. Such printing of stripes of shrinking agent is well-known in the art.

#### Example 2

As starting material, a mixed light weight fabric is used, the warp of which consists of alternating stripes of 6 "nylon" yarns 70 denier single and 10 cotton yarns number 80 single, whereas the weft consists entirely of number 120 single cotton yarn. With a count of 80 threads per inch in the warp and 72 threads per inch in the weft, the width of the stripes formed by the alternating groups of "nylon" yarns and cotton yarns in the direction of the warp are 1.9 mm. and 3.2 mm., respectively. This fabric is boiled and bleached and then color-printed in a stripe pattern, the stripes running parallel to the warp; the width of the colored stripes being 1.25 mm. and the width of the interspace 2.1 mm. For color-printing the color stripe, pigment printing pastes, as represented by the "Aridye" printing colors and for instance described in U. S. Patent 2,364,738, are applied. After fixing of the color print, the fabric is treated for 5 minutes without any tension in a 30° Baumé caustic soda solution, washed with hot water, acidified with dilute sulfuric acid, washed with cold water until neutral and dried on a pin stenter without applying tension warpwise. The result is a crepe-like fabric with a vivid play of the color printed stripes against the unprinted background and with no moiré effect. In this example,

$$\begin{array}{r} (d) \quad (b) \\ 3.2 \quad 2.1 \\ \hline 1.9 = 1.25 \\ (c) \quad (a) \end{array}$$

and

$$\begin{array}{r} (c) + (d) \\ n \approx \frac{1.9 + 3.2}{2} \approx \frac{5.1}{3.35} \approx 1.5; n \approx 3 \\ (a) + (b) \end{array}$$

#### Example 3

A bleached and mercerized light weight fabric such as cotton batiste with 105 ends and 90 picks per inch, the numbers of the warp and weft yarns being 80 and 95, respectively, is printed in a stripe pattern with a vat dyestuff as for instance Ponsol

Violet RR (Color Index 1104). Thereafter a cellulose nitrate lacquer is printed in another stripe pattern, running parallel to the colored stripe pattern, on the backside of the fabric. After drying, the fabric is shrunk with caustic soda solution 36° Bé., treated with dilute sulfuric acid, washed until neutral and stenter dried. The width of the color stripes and the interspaces being 0.8 and 1.6 mm., respectively, and the width of the lacquer printed stripes and the corresponding interspaces being 1.2 and 2.4 mm. The result is a crepe-like fabric with a crisp hand and a vivid play of color printed stripes without any formation of an undesired moiré effect. In this example,

$$\begin{array}{r} (d) \quad (b) \quad (c) + (d) \\ 2.4 \approx 1.6; \quad n \approx \frac{1.2 + 2.4}{2} \approx \frac{3.6}{2.4} \approx 1.5; \quad n \approx 3 \\ 1.2 \approx 0.8; \quad 2 \approx \frac{0.8 + 1.6}{2} \approx \frac{2.4}{2} = 1.2 \\ (c) \quad (a) \quad (a) + (b) \end{array}$$

#### Example 4

A fabric, consisting of number 70 single mixed spun yarns, containing 84 per cent cotton and 16 per cent viscose spun rayon, with 86 ends and 78 picks per inch, is bleached and stenter dried. It is then printed in a stripe pattern with a vat dyestuff as for instance Ciba Scarlet G (Color Index 1228). The width of the printed stripes is 0.5 mm., the distance between two printed stripes is 1.5 mm. After steaming and soaping the fabric is dried, overprinted in another stripe pattern with a thickened 36 per cent caustic soda solution, the width of the caustic printed stripes and the interspaces being 2 mm. each, to locally shrink the fabric. Thereafter, the fabric is treated with dilute sulfuric acid in order to remove the caustic, thoroughly washed until neutral and dried. The resulting fabric shows an interesting crepon effect with a vivid play of color.

#### Example 5

A mixed light weight fabric, the warp of which consists of alternating stripes of 9 threads each of number 70 single gray cotton yarn and 75 denier formaldehyde treated viscose rayon yarn, whereas the weft consists entirely of number 90 single cotton yarn, is boiled and bleached. The count of the fabric is 82 ends and 68 picks per inch; the width of the stripes formed by alternating groups of cotton and formaldehyde treated rayon yarns in the warp is about 3 mm.

The formaldehyde treatment of the viscose yarn is carried out as follows:

Skeins of filament viscose rayon yarn are treated for 15 minutes in an aqueous bath containing per liter: 350 grams of a 38 per cent formaldehyde technical solution and 6 grams of ammonium chloride. Excess liquor is removed by hydroextracting, whereupon the skeins, after being dried at 70° C. are exposed for 15 minutes to a temperature of 120° C. The yarn is then soaped, washed and dried.

The bleached fabric is printed with a colored pigment, as represented by the "Aridye" printing colors and for instance described in U. S. Patent 2,364,738, in a stripe pattern running parallel to the warp, the width of the colored stripes being 1 mm., the distance between two colored stripes being 2 mm. Finally, the fabric is shrunk with 36° Bé. caustic soda solution, treated with dilute sulfuric acid, washed until neutral and dried. The finished fabric shows undulated stripes formed by the groups of viscose yarns superimposed by color printed stripes, which to-

gether apply to the fabric a vivid appearance without any formation of undesired moiré effects.

*Example 6*

The starting material is a fabric, the warp of which consists of alternating stripes of number 38 raw cotton yarn and number 38 cotton yarn which, before weaving, was boiled and treated with a hydrophobing agent such as stearamido-methoxymethylpyridinium chloride, whereas the filling or weft consists entirely of number 44 raw cotton yarn. The count of this fabric is 72 ends and 78 picks per inch, and each alternating group of raw and pre-treated yarn in the warp consists of 9 threads each, thus forming stripes of about 3.2 mm. This fabric, after desizing, is boiled in a bath containing 3 grams per liter of soap and 1 gram of sodium carbonate, and if desired, is bleached in a sodium hypochlorite solution containing 2 grams per liter of active chlorine. Then it is stentered and color printed in a stripe pattern, running parallel to the warp. The width of the color printed stripes and of the interspaces being 1.2 mm. and 2 mm. respectively. For color printing vat dyestuffs as described in Examples 1, 3 and 4 may be used. Finally, the fabric is padded with caustic soda solution 36° Bé., laid down on a conveyor for 5 minutes, where it is allowed to shrink, then treated with dilute sulfuric acid, washed until neutral and dried. The result is a vivid play of color printed stripes on a crepe-like fabric without any formation of undesirable moiré effects.

What we claim is:

1. A process which comprises printing a fabric with parallel spaced colored stripes, said fabric containing sufficient cellulose to produce a crepe effect when treated with a caustic shrinking agent capable of shrinking the cellulose, said fabric having resistant stripes which are resistant to shrinkage, and shrinkable stripes, said shrink resistant stripes and shrinkable stripes being parallel to said colored stripes, shrinking the fabric by applying caustic soda shrinking agent thereto and removing the shrinking agent from the fabric, said colored stripes, shrink resistant stripes and the spaces therebetween being in the relation of both of the equations

$$\frac{d}{c} \approx \frac{b}{a}$$

$$\frac{c+d}{a+b} \approx \frac{n}{2}$$

where  $a$  is the width of a colored stripe,  $b$  is the space between adjacent colored stripes,  $c$  is the width of a shrink resistant stripe,  $d$  is the width of the space between adjacent shrink resistant stripes, and  $n$  is an odd integer except 1.

2. A process which comprises printing a fabric

with parallel spaced colored stripes, said fabric containing sufficient cellulose to produce a crepe effect when treated with a caustic shrinking agent capable of shrinking the cellulose, said

5 fabric having resistant stripes which are resistant to shrinkage, and shrinkable stripes, said shrink resistant stripes and shrinkable stripes being parallel to said colored stripes, shrinking the fabric by applying caustic soda shrinking agent thereto and removing the shrinking agent from the fabric, said colored stripes, shrink resistant stripes and the spaces therebetween being in the relation of both of the equations

$$c=d$$

$$\frac{c+d}{a+b} \approx \frac{n}{2k}$$

where  $a$  is the width of a colored stripe,  $b$  is the space between adjacent colored stripes,  $c$  is the width of a shrink resistant stripe,  $d$  is the width of the space between adjacent shrink resistant stripes, and  $k$  is any integer.

15 3. The process of claim 1 in which  $n$  is equal to 3.

20 4. The process of claim 1 in which the fabric consists of natural cellulose throughout.

5. The process of claim 1 in which a water-insoluble nitro cellulose lacquer resist is printed in stripes on the reverse side of the fabric.

30 6. The process of claim 1 in which a reserve against caustic shrinking agents is printed on the fabric as the spaced shrink resistant stripes.

7. The process of claim 2 in which a reserve against caustic shrinking agents is printed on the fabric as the spaced shrink resistant stripes.

35 8. The process of claim 1 in which the fabric contains cellulose fiber as therein stated, with nylon fibers forming parallel stripes and constituting the shrink resistant stripes.

40 9. The product produced by the process of claim 1.

ERNST WEISS.  
KARL RISCH.

45 REFERENCES CITED

The following references are of record in the file of this patent:

UNITED STATES PATENTS

| 50 | Number    | Name             | Date          |
|----|-----------|------------------|---------------|
|    | 2,171,513 | Heberlein et al. | Aug. 29, 1939 |
|    | 2,200,389 | Finalyson et al. | May 14, 1940  |
|    | 2,319,903 | Huey et al.      | May 25, 1943  |

55 FOREIGN PATENTS

| 60 | Number  | Country       | Date          |
|----|---------|---------------|---------------|
|    | 19,388  | Great Britain | June 29, 1895 |
|    | of 1894 |               |               |
|    | 482,181 | Great Britain | Mar. 24, 1938 |
|    | 494,673 | Great Britain | Oct. 26, 1938 |